

# UNITED STATES PATENT OFFICE.

FRIEDRICH JOHANN HEINRICH ROEWER, OF HAMBURG, GERMANY, ASSIGNOR TO THE  
E. I. DU PONT DE NEMOURS POWDER COMPANY, OF WILMINGTON, DELAWARE, A CORPO-  
RATION OF NEW JERSEY

## PROCESS OF DENSIFYING A NITROHYDROCARBON COMPOSITION.

No. 912,738.

Specification of Letters Patent.

Patented Feb. 16, 1909

Application filed August 13, 1908. Serial No. 448,358.

*To all whom it may concern:*

Be it known that I, FRIEDRICH JOHANN HEINRICH ROEWER, a subject of the Emperor of Germany, residing at Hamburg, Germany, 5 have invented a new and useful Improvement in Processes of Densifying Nitrohydrocarbon Compositions, of which the following is a full, clear, and exact description.

Since trinitrotoluol has lately been used instead of picric acid for loading shells, it has been observed that when fused trinitrotoluol is poured into the shells, after the substance has set, it has a lesser specific gravity than picric acid. A number of propositions have 10 been made for increasing the specific gravity of trinitrotoluol. Thus it has been proposed to increase the density of trinitrotoluol by heavy pressure or by the addition of dinitrotoluol. The pressing is slow and expensive, 15 and moreover, the addition of dinitrotoluol is only a makeshift, as it is considered of great moment to not use any mixture for loading bombs, but only a simple chemical substance.

I have found that nitrotoluol and other 20 suitable nitrohydrocarbons can be obtained of a satisfactory density, as for example 1.6, in a very simple manner and without addition of other compounds, when the substance, heated somewhat above its fusion point, is 25 poured into a receptacle chilled to 0° centigrade, by inserting a paper tube or funnel in the opening of the receptacle, thereby extending the pouring channel vertically, and delivering the substance in through this, per- 30 mitting it to back up in the paper tube, so that the pressure produced by this extra column of material gives a denser casting, in analogy, to metal foundry practice; the ex- 35 cess being removed after the substance is 40 cooled.

In French Patent #369,371 and in British

Patent #19215 of 1906, it is set forth that the nitrohydrocarbons, densified by pressure, may have their density still further increased in a small degree if the mass is chilled during the pressing. But these patents fail to disclose my discovery that a density useful for technical purposes can be produced without the use of pressure.

Having now fully described my invention, 50 what I claim and desire to protect by Letters Patent is:—

1. The process of densifying a nitro-hydrocarbon composition for use in charging projectiles, consisting in introducing the composition, while in a molten condition, into a previously chilled receptacle, substantially as described.

2. The process of densifying a nitro-hydrocarbon composition for use in charging projectiles, consisting in subjecting the same, while in a molten condition, to sudden chilling while maintaining the same free from pressure other than that of the composition itself, substantially as described.

3. The process of densifying a nitro-hydrocarbon composition for use in charging projectiles, consisting in subjecting the same, while in a molten condition, to a sudden chilling and to the pressure of a column of the 70 said composition extending above the part thereof being densified, and maintaining the composition to be densified otherwise free from pressure, substantially as described.

In testimony of which invention, I have 75 hereunto set my hand, at Hamburg, on this 23 day of July, 1908.

FRIEDRICH JOHANN HEINRICH ROEWER.

Witnesses:

HUGO KÖHLING,

ERNEST H. L. MUMMENHOFF.